# EUROPEAN PATENT SPECIFICATION

(11) **EP 0 163 130 B1**
(45) Date of publication and mention of the grant of the patent: **12.07.1989**
(21) Application number: 85105029.4
(22) Date of filing: 25.04.1985
(51) Int. Cl.: G03F 7/26

(54) **Electroforming method and mandrel**
Elektroformungsverfahren und dafür verwendeter Dorn
Procédé d'électroformage et mandrin utilisé

(30) Priority: 30.04.1984 US 605505; 30.04.1984 US 605506
(43) Date of publication of application: 04.12.1985
(73) Proprietor: PPG INDUSTRIES, INC., Pittsburgh Pennsylvania 15272 (US)
(72) Inventor: Postupack, Dennis Sylvester, Natona Heights, Pa. 15065 (US); Pressau, Jean Pierre, Evans City, Pa. 16033 (US); Kenworthy, James Stanely, Rockland, Mass. 02370 (US); Kozinski, Thomas George, South Attleboro, Mass. 02703 (US)
(74) Representative: Sternagel, Hans-Günther, Dr.

(56) References cited:
- EP-A- 0 006 459
- US-A- 3 900 359
- METAL FINISHING ABSTRACTS, vol. 21, no. 5, September/October 1979, pages 320,321; & JP - A - 54 37 038 (DAINIPPON PRINTING K.K.) 27-08-1977

## Description

The present invention relates generally to the art of electroplating, and more particularly to the art of electroforming on a patterned mandrel.

Electroforming of precision patterns, such as those used in optical systems, has been accomplished by several methods. For example, precision mesh patterns have been produced by electroplating onto a master pattern of lines formed by etching or ruling lines into a glass substrate and depositing a conductive material into the etched or ruled lines to form a conductive master pattern for electroplating. A major disadvantage of this method is the limitation on the fineness and precision of etching glass.

Photolithographic techniques have also been used to produce patterned electroforming mandrels. For example, a conductive substrate, such as a polished metal plate, is coated with a layer of photoresist. A patterned photomask is placed over the photoresist, which is then exposed to actinic radiation through the mask, thereby creating a pattern of exposed and unexposed photo- resist which is further developed. Either the exposed or the unexposed portions of the photo- resist are removed, depending on whether a positive or negative pattern is desired, resulting in a conductive pattern on the substrate. An electroplating process is then carried out to form a replica of the conductive pattern which can thereafter be removed from the substrate. This method is also restricted in the uniformity and precision of lines which can be formed, as well as requiring reprocessing of the master pattern after limited usage.

US-A-3,703,450 to Bakewell discloses a method of fabricating precision conductive mesh patterns on a repetitively reusable master plate comprising a conductive pattern formed on a nonconductive substrate and a nonconductive pattern formed in the interstices of the conductive pattern. A reproduction of the master pattern is formed by plating of a conductive pattern onto the master pattern within a matrix defined by the nonconductive pattern. The conductive metal master pattern is typically deposited onto a glass plate by evaporation of a metal such as chromium through a ruled pattern formed on a stencil material. The nonconductive pattern is formed by depositing a layer of photoresist over the conductive pattern coated side of the glass plate. By exposing the photoresist to actinic radiation through the conductive pattern coated substrate, exact registration of the conductive and nonconductive patterns is achieved. The photoresist layer is developed and the exposed portions are removed, leaving a pattern of photoresist over the conductive pattern. A silicon monoxide layer is then deposited over the entire surface of the glass plate, covering both the photoresist/conductive pattern coated portions and the exposed glass portions. Finally, the photoresist overlying the conductive pattern and the silicon monoxide overlying the residual photoresist material are removed, leaving the glass plate coated with a conductive metal pattern and an array of silicon monoxide deposits in the interstitial spaces in the conductive pattern. Replicas of the conductive pattern are then formed by electroplating.

EP-A-006 459 describes an electroforming method wherein a thin metal layer is applied on to a glass substrate and a desired pattern is formed in said metal layer. A photoresist is deposited on said pattern layer. The photoresist is exposed to actinic radiation through the conductive pattern coated substrate and thereafter developed by common methods. The exposed portions are removed and the spaces free of photoresist are filled by galvanically depositing a metal or by depositing a plastic material therein.

It is the object of the invention to provide an alternative process for producing an electroforming mandrel.

This object is attained by a method for producing an electroforming mandrel comprising the steps of: a) providing a first glass substrate which transmits actinic radiation with a pattern which masks the transmission of actinic radiation; b) depositing on a surface of the patterned first substrate a continuous conductive film which transmits actinic radiation, or depositing on a surface of a second glass substrate to be used as the electroforming mandrel a continuous conductive film, wherein the conductive film is selected from the group consisting of indium oxide, tin oxide and mixtures thereof; c) depositing on the conductive film a continuous layer of a photo- resist; d) exposing said photoresist to actinic radiation through said masking first substrate; and e) developing said photo-resist to selectively remove a portion thereof in order to uncover a pattern of the underlying conductive film.

In other embodiments, either the exposed or unexposed photoresist may be removed and the conductive film in the areas underlying the removed photoresist may be etched away. Removing the remaining photoresist exposes a pattern of the conductive film on the glass surface in either a positive or negative image of the pattern on the substrate. The resultant article is employed as a mandrel for the electroforming of metallic parts. The present invention provides an alternative process for producing a heater element grid. A glass substrate transparent to actinic radiation is provided with a desired pattern for the heater element grid to form a photomask. The substrate to be used as the electroforming mandrel is coated with a continuous conductive film which transmits actnic radiation. A continuous layer of photoresist is deposited over the conductive film. The photoresist is exposed to actinic radiation through the photomask, the pattern acting to mask portions of the photoresist from exposure. The photoresist is then developed, and the unexposed portions removed to yield a conductive pattern of the underlying conductive film corresponding to the pattern of the photomask. Alternatively, the exposed portions of the photoresist may be removed to yield a conductive pattern which is a negative image of the pattern of the photomask. The resultant article is employed as a mandrel for the electroforming of a metallic heater element grid. The mandrel is immersed in an electroforming solution, and current is applied to effect the electrodeposition of metal onto the conductive pattern area on the mandrel. When a sufficiently thick deposit is obtained, the remaining photoresist is removed, and the electroformed heating grid is separated from the mandrel.

According to the present invention, a glass plate is provided with a pattern representing the configuration of the article to be produced by electroforming. While the pattern may be formed by a coating, a most preferred embodiment of the present invention utilizes a glass photomask to provide the pattern, preferably a glass photomask having a pattern formed by stain producing metal infused into the glass. Preferred techniques for producing stained glass photomasks are described in detail in US-A-s 4,144,066 and 4,155,735 to Ernsberger.

A continuous conductive film is deposited on the surface of the glass substrate to be used as the electroforming mandrel. The conductive film may be an electroconductive metal oxide selected from tin oxide or indium oxide or mixtures thereof. The conductive film may be deposited by any conventional coating technique such as vacuum deposition, cathode sputtering, chemical vapor deposition or pyrolytic coating techniques. In a most preferred embodiment of the present invention, a conductive film comprising indium oxide is deposited by magnetron sputtering. In a most preferred embodiment of the present invention, a conductive film is sputtered from a cathode comprising 80 to 90 percent indium and 10 to 20 percent tin.

Preferably, the continuous, transparent conductive film is deposited on the stained surface of a stained glass photomask. The conductive film is preferably deposited on the stained surface of the photomask in order to optimize resolution of the pattern.

A continuous layer of photoresist is applied over the conductive film. Any conventional photo- resist with sufficient resolution is acceptable. In a preferred embodiment of the present invention, photoresist in sheet form is laminated to the conductive film. The photoresist is exposed to actinic radiation through the glass plate and conductive film, which transmit sufficient radiation to cure the exposed portions of the photo- resist. The photomask pattern masks portions of the photoresist from exposure, and these portions remain uncured. Following exposure of the photoresist, and a post-curing cycle if necessary, the photoresist is developed. Preferably, the photoresist is contacted with a chemical solution which dissolves and removes the unexposed, uncured portions of the photoresist, thereby providing a pattern of the underlying conductive film which is a positive image of the pattern in the glass photomask. The remaining exposed, cured portions of the photoresist surrounding the conductive pattern form walls within which the electroformed part is subsequently formed. In an alternative embodiment of the present invention a positive working photoresist may be employed to form a conductive film pattern which is a negative image of the photomask pattern.

The resulting mandrel is used for the electroforming of metallic parts replicating the pattern on the conductive film. The glass photomask substrate bearing a conductive film having a pattern defined by the photoresist is contacted with a conventional metal-containing electrodeposition solution. An electrical circuit is established, using the conductive film as the cathode and an electrode of the metal to be deposited as the anode. An electrical potential is applied, and metal is deposited on the conductive film in the pattern defined by the photoresist. Electrodeposition is continued until the desired thickness is obtained for the electroformed part. The substrate bearing the conductive film, photo- resist, and electroformed part is removed from the electrodeposition solution. Separation of the electroformed part from the photomask mandrel may be effected by various means such as alternately heating and chilling. If the part is thick enough, it may be stripped from the mandrel with the photoresist intact. The mandrel is immediately reusable. However, in applications wherein the electroformed part is very thin and/or comprises very fine lines, the remaining photo- resist is first removed, preferably by dissolution. Then the electroformed part is lifted off the photomask mandrel. If the electroformed part is strong enough, it may be simply stripped from the conductive film. However, wherein the electroformed part comprises very fine lines, a preferred method for separating the electroformed part from the photomask mandrel is to contact the electroformed part with a tacky tape to which the part adheres, and to remove the part with the tape. The part is preferably removed from the tape by dissolution of the adhesive.

In a most preferred use according to the present invention wherein the electroformed part is a heating grid comprising very fine lines, a preferred method for separating the electroformed heating element from the mandrel is to remove the photoresist, contact the electroformed part with a polymeric material to which the part adheres, and remove the heating grid element attached to the polymeric material. Preferably, the polymeric material is an interlayer sheet to be laminated to a rigid sheet to form an aircraft transparency. The polymeric material may be a sheet of polyvinyl butyral, a surface of which is chemically treated to soften the surface. The tacky surface is used to pick the heating grid off the mandrel. The polyvinyl butyral sheet is then laminated to a second polymer sheet with the heating grid between them. Various solvents may be used to soften the polyvinyl butyral; diethylene glycol monobutyl ether is preferred.

The present invention will be further understood from the descriptions of specific examples which follow.

### Example I

A glass photomask electroforming mandrel is prepared by coating a glass plate with a photographic emulsion comprising silver halide which is exposed to actinic radiation through a master pattern which defines the shape of the part to be electroformed. Exposed areas of the photographic emulsion form a latent image which is developed by immersion in developing solutions which convert the silver halide to colloidal silver. The coated glass plate is subjected to an electric field which induces migration of the silver ions into the glass. The silver ions are reduced to elemental silver which agglomerates into colloidal, microcrystalline color centers which form a stained pattern within the glass which corresponds with the master pattern of the article to be electroformed. The stained glass surface is then coated with a continuous conductive film by magnetron sputtering of a cathode comprising 90 percent indium and 10 percent tin. The preferred indium oxide film has a surface resistivity less than about 20 ohms per square. A continuous layer of photoresist is applied over the conductive film by laminating a sheet of photoresist to the indium oxide at a temperature of about 113°C (235°F). A photoresist layer having a thickness of about 0.025 millimeter (0.001 inch) is available from Thiokol/Dynachem Corp. of Tustin, California. The photoresist is exposed to actinic radiation (Colight M-218) through the glass photomask for 20 seconds and cured. The photoresist is developed with a solvent which removes the unexposed portions of the photoresist thereby providing a pattern of the underlying indium oxide in the shape of the article to be electroformed. The resultant article is used as an electroforming mandrel in the following process.

### Example II

The glass photomask electroforming mandrel of Example I is prepared for electroforming by sequential dipping into a dilute solution of hydrochloric and nitric acids, and isopropanol, each followed by a water rinse to clean and wet the electroforming surface. The glass photomask is dipped into the electroforming solution several times to completely wet the surface and remove air bubbles before the electroforming process commences. The electroforming solution comprises nickel sulfamate, and is maintained at a temperature of about 43°C (110°F). A cathode contact is applied to the indium oxide film of the glass photomask electroforming mandrel. An anode contact is applied to a depolarized nickel plate. Both the mandrel and the plate are immersed into the nickel sulfamate solution. At a current density of 10 amps per square foot, electroforming proceeds at a rate of 0.025 millimeter (0.001 inch) per 100 minutes. When the electroformed part reaches the desired thickness, the mandrel is removed from the solution, the remaining photoresist is dissolved and removed with sodium hydroxide solution, and the electroformed part is removed from the mandrel with tack tape.

### Example III

A glass photomask is prepared by coating a glass plate with a photographic emulsion comprising silver halide which is exposed to actinic radiation through a master pattern in the shape of the part to be electroformed. Exposed areas of the photographic emulsion form a latent image which is developed by immersion in developing solutions which convert the silver halide to colloidal silver. The coated glass plate is subjected to an electric field which induces migration of the silver ions into the glass. The silver ions are reduced to elemental silver which agglomerates into colloidal, microcrystalline color centers which form a stained pattern within the glass which corresponds with the master pattern of the article to be electroformed. An electroforming mandrel is prepared by coating a glass substrate surface with a continuous conductive film by magnetron sputtering of a cathode comprising 90 percent indium and 10 percent tin. The preferred indium oxide film has a surface resistivity less than 20 ohms per square. A continuous layer of photoresist is applied over the conductive film by laminating a sheet of photoresist to the indium oxide at a temperature of about 113°C. (235°F). A photoresist layer having a thickness of about 0.025 millimeter (0.001 inch) is available from Thiokol/Dynachem Corp. of Tustin, California. The photoresist is exposed to actinic radiation (Colight M-218) through the glass photomask for 20 seconds and cured. The photoresist is developed with a solvent which removes the unexposed portions of the photoresist thereby providing a pattern of the underlying indium oxide corresponding with the pattern in the photomask which in turn corresponds with the master pattern in the shape of the article to be electroformed. The resultant article is used as an electroforming mandrel in the following process.

### Example IV

A glass mandrel about 7.6 by 17.8 centimeters (3 by 7 inches) is prepared as in Example I having a screen pattern comprising lines about 0.03 millimeter (0.0012 inch) wide spaced about 0.56 millimeters (0.022 inches) apart. The mandrel is prepared for electroforming by sequential dipping into a dilute solution of hydrochloric and nitric acids, and isopropanol, each followed by a water rinse to clean and wet the electroforming surface. The glass mandrel is dipped into the electroforming solution several times to completely wet the surface and remove air bubbles before the electroforming process commences. The electroforming solution comprises nickel sulfamate, and is maintained at a temperature of about 43°C (110°F). A cathode contact is applied to the indium oxide film of the glass electroforming mandrel. An anode contact is applied to a depolarized nickel plate. Both the mandrel and the plate are immersed into the nickel sulfamate solution. At a current density of 10 amps per square foot, electroforming proceeds at a rate of 0.025 millimeter (0.001 inch) per 100 minutes. When the electroformed part reaches the desired thickness, about 0.013 mm (0.0005 inches), the mandrel is removed from the solution. The remaining photoresist is dissolved and removed with sodium hydroxide solution at about 66°C. (150°F). The electroformed heating grid is removed from the mandrel by contacting the surface with a sheet of polyvinyl butyral, the contacting surface of which has been treated with diethylene glycol monobutyl ether to produce an adhesive surface. As the polyvinyl butyral sheet is pulled away from the mandrel, the grid remains attached to the tacky surface of the polyvinyl butyral. To form a heatable interlayer, the polyvinyl butyral sheet bearing the heating grid is laminated to another polymeric sheet with the heating grid between the sheets.

### Example V

An optical grid is produced by electroforming as in Example II, except that the conductive pattern on the mandrel comprises finer lines more closely spaced. An optical grid is produced comprising lines about 0.025 millimeter (0.001 inch) wide spaced about 0.076 millimeter (0.003 inch) apart.

The above examples are offered to illustrate the present invention. Various modifications are included within the scope of the present invention. For example, metallic substrates may be used for the electroforming mandrel, and other metals may be deposited by electroforming, such as copper, iron, lead, tin and zinc. The electroformed elements of the present invention need not be grid patterns, but may be produced in any shape or configuration, limited only by the artwork. The scope of the present invention is defined by the following claims.

## Claims

1. A method for producing an electroforming mandrel comprising the steps of:
a) providing a first glass substrate which transmits actinic radiation with a pattern which masks the transmission of actinic radiation;
b) depositing on a surface of the patterned first substrate a continuous conductive film which transmits actinic radiation, or depositing on a surface of a second glass substrate to be used as the electroforming mandrel a continuous conductive film, wherein the conductive film is selected from the group consisting of indium oxide, tin oxide and mixtures thereof;
c) depositing on the conductive film a continuous layer of a photoresist;
d) exposing said photoresist to actinic radiation through said masking first substrate; and
e) developing said photoresist to selectively remove a portion thereof in order to uncover a pattern of the underlying conductive film.

2. A method according to claim 1, wherein the glass substrate is provided with a masking pattern by means of a stain pattern within the glass.

3. A method according to claim 1, wherein the conductive film is deposited by magnetron sputtering.

4. A method according to claim 1, wherein the photoresist is applied by laminating a sheet of photoresist to the conductive film.

5. A method according to claims 1 to 4, wherein the photoresist is developed by contacting it with a solvent which removes the uncured portionsofthe photoresist.

6. Use of the electroforming mandrel according to any of the preceding claims for electroforming a metallic article.

## Patentansprüche

1. Verfahren zum Herstellen einer Form für Galvanoplastik mit den Schritten
a) Versehen eines ersten, aktinische Strahlung durchlassenden Glasträgers mit einem für aktinische Strahlung undurchlässigen Muster;
b) Aufbringen eines durchgehenden leitenden Filmes, der aktinische Strahlung durchläßt, auf die Oberfläche des mit einem Muster versehenen ersten Trägers oder Aufbringen eines durchgehenden leitenden Filmes auf die Oberfläche eines zweiten Glasträgers, der als Form für Galvanoplastik verwendet werden soll, wobei der leitende Film aus der Gruppe bestehend aus Indiumoxid, Zinnoxid und Mischungen derselben ausgewählt ist;
c) Aufbringen einer durchgehenden Schicht eines Photoresist auf den leitenden Film;
d) Aussetzen des Photoresist aktinischer Strahlung durch den abdeckenden ersten Träger; und
e) Entwickeln des Photoresist, um ausgewählte Stellen desselben zu entfernen, so daß ein Muster im darunterliegenden leitenden Film nicht mehr abgedeckt ist.

2. Verfahren nach Anspruch 1, dadurch gekennzeichnet, daß das undurchlässige Muster auf dem Glasträger durch Einfärben des Glases erzeugt wird.

3. Verfahren nach Anspruch 1, dadurch gekennzeichnet, daß der leitende Film durch Magnetronkathodenzerstäubung erzeugt wird.

4. Verfahren nach Anspruch 1, dadurch gekennzeichnet, daß der Photoresist durch Laminieren einer Folie des Photoresist auf den leitenden Film aufgebracht wird.

5. Verfahren nach Ansprüchen 1-4, dadurch gekennzeichnet, daß der Photoresist durch Inberührungbringen mit einem Lösungsmittel, das nicht gehärtete Teile des Photoresist entfernt, entwickelt wird.

6. Verwendung der galvanoplastischen Form nach jedem der vorstehenden Ansprüche zum galvanoplastischen Ausbilden eines metallischen Gegenstandes.

## Revendications

1. Procédé de fabrication d'un mandrin d'électroformage, comprenant les étapes consistant à:
a) munir d'un dessin qui masque la transmission de radiations actiniques un premier substrat de verre qui transmet les radiations actiniques;
b) déposer, sur une surface du premier substrat muni du dessin, un film conducteur continu qui transmet les radiations actiniques ou déposer un film conducteur continu sur une surface d'un second substrat de verre destiné à être utilisé comme mandrin d'électroformage, le film conducteur étant choisi dans le groupe constitué par l'oxyde d'indium, l'oxyde d'étain et des mélanges de ceux-ci;
c) déposer sur le film conducteur une couche continue d'une matière photorésistante;
d) exposer cette matière photorésistante aux radiations actiniques à travers le premier substrat de masquage; et
e) développer la couche phosorésistante pour en éliminer sélectivement une partie, afin de mettre à nu un dessin du film conducteur sous- jacent.

2. Procédé selon la revendication 1, dans lequel le substrat de verre est muni d'un dessin de masquage au moyen d'un dessin par taches dans le verre.

3. Procédé selon la revendication 1, dans lequel le film conducteur est déposé par pulvérisation par magnétron.

4. Procédé selon la revendication 1, dans lequel la matière photorésistante est appliquée par superposition d'une feuille de matière photorésistante sur le film conducteur.

5. Procédé selon l'une quelconque des revendications 1 à 4, dans lequel la couche photorésistante est développée par sa mise en contact avec un solvant qui élimine les parties non durcies de la couche photorésistante.

6. Utilisation du mandrin d'électroformage selon l'une quelconque des revendications 1 à 5 pour l'électroformage d'un article métallique.
